

## UNITED STATES PATENT OFFICE

ROBERT T. WOOD, OF LAKewood, AND HAROLD H. BLOCK, OF CLEVELAND, OHIO, AS  
SIGNORS TO AMERICAN MAGNESIUM CORPORATION, OF PITTSBURGH, PENNSYLVANIA, A CORPORATION OF NEW YORK

## MAGNESIUM BASE ALLOY

No Drawing. Application filed August 6, 1931. Serial No. 555,532.

This invention relates to magnesium base alloys and is directed to the development of alloys of this class characterized by a high resistance to corrosion.

The specific gravity of magnesium is only about two thirds of that of aluminum and this constitutes a decided advantage in favor of magnesium and its alloys. For this reason efforts are constantly being exerted to improve magnesium base alloys in those respects in which aluminum base alloys now have the advantage, for instance, corrosion resistance. While many articles made from magnesium base alloys are now in daily service, it is desirable that alloys be produced which will be able to satisfactorily resist conditions more severe than usual, for instance constant exposure to salt-air or aggravated atmospheric conditions, without danger of failure from corrosion.

The principal object of the invention is the production of magnesium base alloys of higher corrosion resistance than characterizes the useful magnesium base casting alloys which have heretofore been available.

An important object of the invention is to provide magnesium base alloys of high corrosion resistance with physical properties adequate to fulfill commercial needs. The terms "magnesium base alloys" and "magnesium alloys" as used in this specification and the appended claims are to be understood as meaning alloys containing more than 50 per cent of magnesium.

The magnesium-aluminum-manganese alloy widely used commercially in this country for casting purposes exhibits physical properties which are comparatively excellent and are amenable to improvement by suitable heat treatments. Its combination of properties has been the best heretofore obtainable in a general purpose casting alloy, but under severe conditions it is noticeably subject to corrosion. Various protective coatings more or less beneficial have been devised and applied to the alloy to improve its corrosion resistance. Protective coatings, however, only attempt to counteract an innate evil whereas the alloys which form the subject of our present invention are in-

herently resistant to corrosion and exhibit that important property to a marked extent even without protective coatings of any sort.

In the course of our investigations, wherein alloys were compounded of various constituents and tested for physical properties and corrosion resistance, we found that magnesium alloys containing varying amounts of tin, zinc and cadmium with or without other constituents are characterized by satisfactory physical properties and corrosion resistance. The alloys may contain from 0.1 per cent to 15.0 per cent tin, from 0.1 per cent to 5.0 per cent zinc, and from 0.1 per cent to 20.0 per cent cadmium. The amounts of these constituents may vary widely but when all are present their cooperative effect is highly desirable. Our experience also indicates that whereas aluminum as an alloy base is highly resistant to corrosion, its presence in a magnesium base alloy does not, in general, improve the property mentioned and in some cases may even increase the susceptibility of the alloy to corrosion.

In testing our new alloys we have subjected the same to particularly aggravated corrosive conditions. One such test which has been standardized for the purpose of comparing different alloys consists in repeatedly immersing the alloy in a 3 per cent aqueous solution of sodium chloride alternating with exposures to the atmosphere. This test is chosen not only because it is more severe than ordinary service conditions but also for the reason that it gives numerically measurable corrosion effects in a fairly short time. In this test a duration of 40 hours has been adopted as a standard.

In carrying out the test a number of tensile specimens identical as to composition and casting conditions were divided into two groups and one group was tested for physical properties, such as tensile strength and elongation. The other group was put through the alternate immersion test already described and was tested at the conclusion of the procedure. The difference between the average strengths of the two groups is a measure of the deterioration from corrosion.

The commercial magnesium-aluminum-

55  
60  
65  
70  
75

75

75  
80  
85

90  
95  
100

manganese casting alloy, mentioned above, at the end of 40 hours of test, had lost between 50 per cent and 60 per cent of its original strength. On the other hand, a magnesium base alloy containing tin 2.03 per cent, zinc 5.20 per cent, and cadmium 2.23 per cent, lost under the same conditions only 15 per cent of its original strength. At the start the two alloys had a tensile strength of 25,000 and 22,800 pounds per square inch, respectively,

10 and at the close of the test the tensile strengths were 12,000 and 18,380 pounds per square inch. Our alloy, therefore, at the start of the test was somewhat inferior in strength but at 15 the end showed about 50 per cent improvement over the prior alloy. Further improvement in our alloy was effected by heat treatment, the heat treated specimen losing about 11 per cent of its original strength.

20 We have also found that the presence of one or more of the elements lead, manganese and mercury effects a further improvement. The lead may be introduced in amounts from 0.1 per cent to 10.0 per cent, the manganese from 0.1 per cent to 5.0 per cent, and the mercury to a lesser extent in the neighborhood 25 of about 0.1 per cent to 0.5 per cent. Although manganese when added in amounts from 0.1 to 5.0 per cent gives beneficial results, the preferred results are obtained when 30 the alloy contains not less than about 0.5 per cent.

35 For example, a magnesium alloy containing tin 3.1 per cent, zinc 3.3 per cent, cadmium 3.3 per cent, and lead 3.2 per cent, subjected to the above test, showed a loss of 13 per cent of original tensile strength, which was 24,000 pounds per square inch in the "as cast" condition. After heat treatment the loss was only 40 7.5 per cent of the original strength.

45 As an example of the beneficial effect of lead and manganese, a magnesium alloy containing tin 2.11 per cent, zinc 2.3 per cent, cadmium 2.00 per cent, lead 2.07 per cent, and manganese 1.74 per cent, with a tensile 50 strength of 24,200 pounds per square inch as cast, and 27,700 pounds after heat treatment, showed a loss of 12 per cent of its original strength in the as-cast condition and in the heat treated condition only 9.5 per cent.

55 As an example of the beneficial effect of the addition of manganese alone, a magnesium alloy containing tin 5.0 per cent, zinc 2.0 per cent, cadmium 2.0 per cent, and manganese 1.0 per cent, lost only 10 per cent of its original strength as cast.

60 As an example of the beneficial effect of the addition of lead and mercury, a magnesium alloy containing tin 2.00 per cent, zinc 2.00 per cent, cadmium 1.59 per cent, lead 1.59 per cent, and mercury 0.20 per cent, with an as-cast strength of 24,300 pounds per square inch, showed a loss of only 7 per cent of its original strength.

65 As the result of numerous tests on mag-

nesium base alloys containing tin, zinc and cadmium in combination with other previously selected elements, we have selected a preferred alloy of the following composition as having an exceptionally good combination of casting and corrosion resistant qualities together with satisfactory mechanical properties:

|           |            |    |
|-----------|------------|----|
| Tin       | 6 per cent | 75 |
| Cadmium   | 1 per cent |    |
| Zinc      | 1 per cent |    |
| Manganese | 1 per cent |    |
| Magnesium | balance    |    |

80 As a result of a large number of tests we have determined that the advantageous effects of the alloying elements herein disclosed and claimed are observable over a wide range of composition in the case of each element. The corrosion test used in each case was the 85 same as that heretofore described, in which the prior magnesium-aluminum-manganese casting alloy hitherto found most advantageous suffered a loss in strength of from 50 to 60 per cent. The following are the results of some of these tests:

90 A sand cast magnesium base alloy containing 2 per cent cadmium, 2.0 per cent lead, 2.0 per cent zinc, and 15.0 per cent tin showed a loss of only 6.0 per cent of its original strength after the corrosion test.

95 A sand cast magnesium base alloy containing 2.0 per cent cadmium, 2.0 per cent lead, 2.0 per cent tin, and 5.0 per cent zinc showed a loss in strength of only 7.0 per cent.

100 A sand cast magnesium base alloy containing 20.0 per cent cadmium, 2.0 per cent lead, 2.0 per cent tin, and 2.0 per cent zinc showed a loss in strength of only 5.0 per cent.

105 A sand cast magnesium base alloy containing 2.0 per cent cadmium, 10.0 per cent lead, 2.0 per cent tin, and 2.0 per cent zinc showed a loss in strength of only 9.0 per cent.

110 A sand cast magnesium base alloy containing 2.0 per cent cadmium, 3.6 per cent manganese, 2.0 per cent lead, 2.0 per cent tin and 2.0 per cent zinc showed a loss in strength of only 4.0 per cent.

115 In compounding the alloy, the various constituents may be added by methods well known to the art, such as by the addition in the pure state to the molten magnesium or by the use of so-called "rich alloys" or "hardeners" of two or more of the alloying elements. We do not wish to stipulate a set 120 technique since practice usually varies with the equipment and personnel of the different foundries.

125 Our alloys are especially useful for casting purposes, and may be subjected, in the cast and also in the worked state, to the various heat-treatments designed for the improvement or alteration of one or more of their physical properties.

130 Our present application is a continuation

in part of our earlier application Serial No. 504,430, filed December 23, 1930.

What we claim is—

1. A magnesium base alloy containing 0.1 per cent to 15.0 per cent tin, 0.1 per cent to 5.0 per cent zinc, and 0.1 per cent to 20.0 per cent cadmium.
2. A magnesium base alloy containing 0.1 per cent to 15.0 per cent tin, 0.1 per cent to 5.0 per cent zinc, 0.1 per cent to 20.0 per cent cadmium, and 0.1 per cent to 10.0 per cent lead.
3. A magnesium base alloy containing 0.1 per cent to 15.0 per cent tin, 0.1 per cent to 5.0 per cent zinc, 0.1 per cent to 20.0 per cent cadmium, and 0.5 per cent to 5.0 per cent manganese.
4. A magnesium base alloy containing 0.1 per cent to 15.0 per cent tin, 0.1 per cent to 5.0 per cent zinc, 0.1 per cent to 20.0 per cent cadmium, and 0.1 per cent to 0.5 per cent mercury.
5. A magnesium base alloy containing 0.1 per cent to 15.0 per cent tin, 0.1 per cent to 5.0 per cent zinc, 0.1 per cent to 20.0 per cent cadmium, 0.1 per cent to 10.0 per cent lead, and 0.5 per cent to 5.0 per cent manganese.
6. A magnesium base alloy containing 0.1 per cent to 15.0 per cent tin, 0.1 per cent to 5.0 per cent zinc, 0.1 per cent to 20.0 per cent cadmium, 0.1 per cent to 10.0 per cent lead, and 0.1 per cent to 0.5 per cent mercury.
7. A magnesium base alloy containing 0.1 per cent to 15.0 per cent tin, 0.1 per cent to 5.0 per cent zinc, 0.1 per cent to 20.0 per cent cadmium, 0.1 per cent to 10.0 per cent lead, 0.5 per cent to 5.0 per cent manganese, and 0.1 per cent to 0.5 per cent mercury.
8. A magnesium base alloy containing 0.1 per cent to 15.0 per cent tin, 0.1 per cent to 5.0 per cent zinc, 0.1 per cent to 20.0 per cent cadmium, 0.5 per cent to 5.0 per cent manganese, and 0.1 per cent to 0.5 per cent mercury.
9. A magnesium base alloy containing about 6 per cent tin, about 1.0 per cent manganese, about 1.0 per cent zinc, and about 1.0 per cent cadmium.
10. A magnesium base alloy containing 0.1 per cent to 15.0 per cent tin, 0.1 per cent to 5.0 per cent zinc, 0.1 per cent to 20.0 per cent cadmium, 0.1 per cent to 10.0 per cent lead, 0.1 per cent to 5.0 per cent manganese, and 0.1 per cent to 0.5 per cent mercury.
11. A magnesium base alloy containing 0.1 per cent to 15.0 per cent tin, 0.1 per cent to 5.0 per cent zinc, 0.1 per cent to 20.0 per cent cadmium, 0.1 per cent to 5.0 per cent manganese, and 0.1 per cent to 0.5 per cent mercury.

In testimony whereof we hereto affix our signatures.

ROBERT T. WOOD.  
HAROLD H. BLOCK.